

# UNITED STATES PATENT OFFICE.

JEROME ALEXANDER, OF NEW YORK, N. Y.

## ADHESIVE AND PROCESS OF MAKING SAME.

1,300,097.

Specification of Letters Patent.

Patented Apr. 8, 1919.

No Drawing. Continuation of application Serial No. 849,864, filed July 9, 1914. This application filed November 30, 1917. Serial No. 204,762.

To all whom it may concern:

Be it known that I, JEROME ALEXANDER, a citizen of the United States, residing in the borough of Manhattan, city, county, and State of New York, have invented certain new and useful Improvements in Adhesives and Processes of Making the Same, of which the following is a specification.

This invention relates to a non-gelatinizing glue-derived adhesive characterized by the property when dry of being readily soluble in cold water, and to the process of producing same.

Heretofore, animal glue adhesives in liquid form have not been practicable articles of commerce because of the tendency of the glue solution to gelatinize. It has been customary, therefore, to manufacture glue in dry form, and to ship and sell it as piece glue. For useful application, the preparation of such glue requires the mixing of it with heated water and stirring it therein until dissolved and liquid. Stirring it into water at ordinary temperatures is ineffective, since glue does not dissolve in cold water, and it is therefore necessary to heat or boil such a mixture.

With my improved adhesive the gelatinization of the glue in solution is controlled as desired and may either be totally inhibited or partially so, dependent upon the relative quantity of gel-inhibitant employed. My product may be marketed therefore as a ready-mixed liquid glue if desired, or as a dry glue. As a dry product, the solubility of the glue is so increased by the presence of the gel-inhibiting agent that it readily dissolves in water at ordinary temperatures. Such increased solubility results primarily from the method of treatment above described, whereby the gelatinization of the glue is controllably prevented, and is further augmented by the use, as a gel-inhibitant, of a substance having a high water-affinity, and preferably one that is also exothermic.

My improved process essentially consists in the reduction of animal derived glue to a finely divided form and mixing therewith a finely divided dry, inorganic gel-inhibiting substance. The resultant adhesive has the capacity of being readily dissolved by water at ordinary temperatures when mixed therewith, since the tendency to gelatiniza-

tion is prevented and the water or similar solvent is thereby permitted to continue to act upon the glue particles. It has the further capacity when dissolved by water of remaining fluid, due to the inhibition of gelatinization. The dry product is preferable as an article of commerce both because cheaper to package, since liquid glue such as fish glue has to be so shipped as to prevent leakage, and because cheaper to ship, since the increased bulk and weight due to the large fluid content, greatly increases the cost of transportation. It is also preferable because it may be readily used since it can be dissolved without heat. The liquid glue obtained therefrom is capable of the uses for which liquid glue is generally adapted, either alone or in combination with other substances, as, for example, for sizing and the like purposes. The advantage of partial gel-inhibition renders it particularly adaptable for use in the production of calcimine, since by the use of a less quantity of gel-inhibitant, partial gelatinization may be permitted, so that the whiting employed in the manufacture of calcimine will not settle out but will be held in suspension in the mixture by the controlled gelatinization of the glue constituent.

The proportion of gel-inhibitant to be employed with any specific kind of glue will vary according to the jelly-strength of the glue, the rule being that the higher the jelly-strength the larger the relative percentage of gel-inhibitant required to cause the adhesive produced, when mixed with a given amount of water, to remain fluid at a given temperature.

In practising my invention, the principle of gel-inhibition may be applied either by a wet or a dry process, examples of both of which are selected, as follows:

### *The wet process.*

Dissolve a suitable inorganic substance in water until it approximates a saturated solution; dissolve a dry commercial animal glue in sufficient warm water to make a fluid solution therewith; mix these resultant solutions thoroughly; evaporate the water from the mixture, and comminute the residue.

### *The dry process.*

Pulverize a suitable metallic salt; sep-

arately pulverize a commercial glue; and mechanically mix the powdered substances intimately.

As will be understood from the foregoing, 5 the essential steps of either process are the reduction of glue and the gel-inhibiting substance each to a finely divided form and the intimate mixture of the two.

As a specific example of materials and 10 proportions, the following is given:

Grind or otherwise reduce to a finely divided form a commercial animal glue. Assuming such glue to have a jelly-strength of 50, which corresponds to the grade commonly known as Cooper's 1 $\frac{1}{4}$ , take 50 parts thereof by weight.

Granulate or otherwise finely divide calcium chlorid of commercial quality, and take 17 parts thereof by weight. Mechanically mix the two substances intimately. 20 This mixture will then be soluble in water at 20° C. and will pass entirely into solution with 50 parts of water by weight when combined with the dry mixture.

25 Since my process is directed to the treatment of glue so as to arrest its gelatinizing tendency, in practising this process I can employ any inorganic substance which acts as a gel-inhibitant to control the gel formation.

Throughout this specification and the claims defining my invention, the term "gel-inhibitant" is employed as descriptive of such dry inorganic substance as is characterized by the property of preventing the formation of gel in an animal glue solution, or whose presence in a solution of such glue has the power of decreasing the jelly-strength thereof. Such gel-inhibitant may 35 be employed in such proportion as to prevent gelatinization of glue in solution, or in less proportion to permit partial gelatinization upon standing. Since the solubility of animal glue varies with its strength of gelatinization, other conditions being the same, glues of low jelly-strength liquefy at lower temperatures than those of high jelly-strength. My invention therefore contemplates the addition to an animal glue of any 40 inorganic substance which prevents the formation of gel in a glue solution, thus preserving the initial fluidity thereof; or the addition of such quantity as will limit such formation to the desired degree. The adhesive thus produced is substantially unaffected as to the other properties of the particular kind and grade of glue employed. The solubility, however, is at the maximum, and when mixed with a solvent the fluidity 45 of the mixture varies according to the degree of the inhibition of the tendency to gelatinization.

The class of substances having the highest functional efficiency as gel-inhibitants now known to me are certain of the metallic salts,

to wit, those characterized by the property of having a marked affinity for water. This property is itself of especial value, since it facilitates the dissolution of the glue particles which tend to break up more readily 70 as the action of water thereupon, even at ordinary temperatures, is more vigorously exercised. Preferably I employ such of these metallic salts as are further characterized by the additional property of developing 75 heat upon the addition of water. This last-named property still further assists in dissolving the glue by reason of the rise in temperature resulting in the nascent solution. Certain of the gel-inhibiting metallic salts 80 which have the property of a marked affinity for water are, however, endothermic, as, for example, sodium nitrate. Such endothermic salts lack the added advantage accompanying the use of those preferred metallic salts 85 which the exothermic, such, for example, as the chlorids of calcium, zinc, or magnesium. Of these metallic chlorids I recommend calcium chlorid for commercial reasons, as it is readily procurable at low cost. 90

The specific products resulting from the employment of the exothermic metallic chlorids, and particularly calcium chlorid, constitute the subject-matter of my companion application Serial Number 849,864, filed July 9, 1914, of which this application is in part a continuation.

Having thus described my invention, I claim:

1. The process of producing a dry adhesive soluble in water at ordinary temperatures consisting in finely dividing glue, separately finely dividing a gel-inhibitant, and intimately mixing the two substances while each is in a finely divided state. 105

2. The process of producing a dry adhesive soluble in water at ordinary temperatures, consisting in finely dividing glue, separately finely dividing a gel inhibiting substance having a marked affinity for water, 110 and intimately mixing the two substances while each is in a finely divided state.

3. The process of producing a dry adhesive soluble in water at ordinary temperatures, consisting in finely dividing glue, separately finely dividing a gel-inhibiting exothermic substance, and intimately mixing the two substances while each is in a finely divided state.

4. The process of producing a dry adhesive soluble in water at ordinary temperatures consisting in finely dividing glue, separately finely dividing a gel-inhibiting exothermic substance having a marked affinity for water, and intimately mixing the two substances while each is in a finely divided state.

5. The process of producing a dry adhesive soluble in water at ordinary temperatures comprising the following steps: finely

- dividing glue; finely dividing a metallic salt characterized by the properties of high affinity for water and capacity for limiting gel-formation in a glue solution; and mechanically mixing the resultant fine divisions of glue and metallic salt intimately. 5
6. The process of producing a dry adhesive soluble in water at ordinary temperatures, comprising the following steps: 10 finely dividing glue; separately finely dividing a metallic salt characterized by the capacity of tending to inhibit gel-formation in a glue solution; and mechanically mixing the resultant fine divisions of glue and metallic salt intimately. 15
7. The process of producing a dry adhesive soluble in water at ordinary temperatures, comprising the following steps: finely dividing glue; finely dividing an exothermic 20 metallic salt characterized by the capacity of tending to inhibit gel-formation in a glue solution; and mechanically mixing the resultant fine divisions of glue and metallic salt intimately. 25
8. The process of producing a dry adhesive soluble in water at ordinary temperatures, comprising the following steps: finely dividing glue; finely dividing an exothermic metallic salt characterized by the properties 30 of high affinity for water and capacity for limiting gel-formation in a glue solution; and mechanically mixing the resultant fine divisions of glue and metallic salt intimately. 35
9. The method of controlling the solubility of dry glue consisting in intimately mixing therewith a finely divided inorganic gel-inhibitant and varying the quantity thereof in proportion to the jelly-strength 40 of the glue and to the degree of solubility desired. 45
10. The method of controlling the tendency to gel-formation in animal glue solutions consisting in ascertaining the jelly-strength of the glue and in intimately mixing therewith a finely divided inorganic gel-inhibitant in quantity predetermined by
- such jelly-strength, and such that the solution will remain fluid at a given temperature. 50
11. A dry adhesive composed of glue and a substance adapted to control the gelatinization of the glue to a predetermined degree. 55
12. A finely divided dry adhesive soluble in water at ordinary temperatures composed of glue and an exothermic substance adapted to control the gelatinization of the glue to a predetermined degree. 60
13. A finely divided dry adhesive soluble in water at ordinary temperatures composed of glue and a substance having a high affinity for water and adapted to control the gelatinization of the glue to a predetermined degree. 65
14. A dry adhesive soluble in water at ordinary temperatures composed of finely divided glue and a finely divided exothermic substance having a high affinity for water and adapted to control the gelatinization of the glue to a predetermined degree. 70
15. A dry adhesive composed of finely divided glue and a metallic salt adapted to control the gelatinization of the glue to a predetermined degree. 75
16. A dry adhesive soluble in water at ordinary temperatures composed of finely divided glue and an exothermic metallic salt adapted to control the gelatinization of the glue to a predetermined degree. 80
17. A dry adhesive soluble in water at ordinary temperatures composed of finely divided glue and a metallic salt having a high affinity for water and adapted to control the gelatinization of the glue to a predetermined degree. 85
18. A finely divided dry adhesive soluble in water at ordinary temperatures composed of finely divided glue intimately mixed with a finely divided exothermic salt having a high affinity for water and adapted to control the gelatinization of the glue to a predetermined degree. 90

JEROME ALEXANDER.